

## UNITED STATES PATENT OFFICE.

OTHO M. OTTE, OF TARENTUM, PENNSYLVANIA, ASSIGNEE, BY MESNE ASSIGNMENTS,  
TO ALLEGHENY STEEL COMPANY, OF BRACKENRIDGE, PENNSYLVANIA, A CORPO-  
RATION OF PENNSYLVANIA.

## METHOD OF MAKING SHEETS.

No Drawing.

Application filed November 10, 1924. Serial No. 749,030.

This invention relates to the manufacture of high grade steel or alloy sheets and one of the objects of this invention is to provide a method by means of which sheets suitable for deep stamping operations and having a high surface finish free from scale can be readily and cheaply manufactured.

The method is applicable to the manufacture of high grade sheets of low carbon steel and is particularly applicable to the manufacture of high grade sheets from alloys in which it is difficult to remove the scale formed during hot rolling and during annealing at high temperatures.

15 The alloys in the working of which the method of this invention is particularly valuable are those commonly known to-day as stainless iron alloys. These are made from various compositions of iron and chromium and have a relatively low carbon content and in some cases contain silicon and other metalloids.

20 The chromium content generally varies from 8% to 60% with the carbon content as low as practicable, generally ranging from .02% to .14%.

In carrying out this invention, any of the standard sheet mill methods may be utilized and my invention primarily consists in preventing the formation of scale during rolling and during annealing by providing a protective metallic envelope for what may be termed the stock which may either be the sheet bars or the rough-downs. This protective envelope, after the sheets have been finished to gauge and annealed is removed.

35 The protective envelope may, and preferably does consist of a coat of nickel electrolytically deposited.

40 If the protective envelope is to be applied to the sheet bars, the bars are first thoroughly pickled to remove the scale (in some cases, the bars may be ground to remove the scale) and are then given a relatively thick coat of nickel by means of any of the well-known electrolytic processes. The plated sheet bars can be converted into sheets by any of the standard sheet mill methods and, after the finished sheets are annealed at tem-

peratures sufficiently high to render them 50 soft enough for deep stamping operations, the protective envelope is removed. If nickel is the envelope then the sheets are treated with any suitable nickel stripper among those now on the market. If a protective 55 coat other than nickel is used, a stripper must be used (for removing such coat from the finished sheets) that is capable of stripping such metal without harming the surface of the sheets therebeneath.

60 I have found that if sheet bars produced from ingots of iron chromium alloys relatively low in carbon and in which the chromium content is between 11% and 21% are thoroughly pickled to remove the scale, are 65 then plated with a relatively heavy plate of nickel I can produce from such plated bars sheets that are suitable for deep stamping operations, that have a high surface finish and that are extremely resistant to corrosion. 70

If it is desired to plate the rough-downs instead of the sheet bars, the rough-downs must first be thoroughly pickled before plating.

75 The nickel protective coat, during the manufacture of the sheets, either from the plated sheet bars or from the plated rough-downs, of course decreases in thickness as the gauge is lessened, but always preserves the alloy or steel underneath and, serving as a 80 nickel envelope, prevents the sheets from scaling during hot rolling and also during annealing at high temperatures.

85 After the sheets have been stripped of the protective envelope, they may be treated in any manner desired, either by light cold rolling or by buffing or polishing. The sheets, however, when the nickel coat is removed, can be given a fine lustrous surface by buffing and being free from scale, the surface is 90 smooth and of uniform color and resists corrosion to a high degree. I find that buffing is all that is generally required to give the sheets a permanent and lustrous sheen.

Having thus described my invention, what 95 I claim is:—

The method of making lustrous sheets from an iron chromium alloy, in which the

chromium content is in excess of 8%, which consists in forming sheet bars from such alloy, in roughing down said bars, in pickling the rough-downs to remove the scale, in plating the pickled rough-downs with a protective coat of high melting point metal, in rolling the plated rough-downs to length and

in annealing the same, in dissolving off the plating and then in buffing the sheets.

In testimony whereof, I have hereunto 10  
subscribed my name this 8th day of November, 1924.

OTHO M. OTTE.